

Patented Feb. 28, 1928.

1,660,409

# UNITED STATES PATENT OFFICE.

FREDERICK M. BECKET, OF NEW YORK, N. Y., ASSIGNOR TO ELECTRO METALLURGICAL COMPANY, A CORPORATION OF WEST VIRGINIA.

## ZIRCONIUM-MANGANESE STEEL.

No Drawing.

Application filed July 9, 1926. Serial No. 121,495.

This invention relates to manganese steels and comprises a steel which contains manganese in excess of those proportions which may be regarded as normal for plain carbon steels, and which also contains zirconium or is characterized by the modifying effects of zirconium thereon.

Practically all steels contain manganese in small proportions, say up to 0.5% or some what higher, the manganese being usually introduced as a deoxidizer and to counteract the red-shortness due to sulfur, and having in these small proportions little or no significance as an alloying metal. True manganese steels of the Hadfield type, containing around 12% or 13% manganese and characterized by extraordinary toughness and hardness are also well known. More recently steels of manganese content intermediate these extremes have come into use, the manganese usually lying between 1% and 2%, and the carbon varying from fractional quantities up to about 1%. Such steels, especially those of relatively low carbon content (for example around 0.3% carbon), possess high tensile strength and toughness.

It is now well known that zirconium, added in small proportions, say 0.15% to 0.50%, has a marked beneficial effect upon certain steels, both of the plain carbon and alloy types. With certain other steels, on the contrary, no beneficial action of zirconium has been observed.

My investigations of the manganese steels have disclosed a pronounced beneficial action of zirconium in the case of those steels above mentioned which contain manganese in the proportions of about 1% to 2%, or slightly below or above these limits, carbon being below about 1%. So far as my investigations have shown, this marked action of zirconium, which is best evidenced by the increase in shock resistance of the steels as measured by the Izod test, is characteristic of these particular manganese steels. Similar effects have not been observed with manganese either substantially above or substantially below the above range. The optimum results as regards shock resistance have been obtained with steels containing carbon around 0.3% with manganese about 1.25%, although my invention is of course not restricted to this particular composition.

The effects of zirconium on the physical properties of certain steels within the range contemplated by this invention are illustrated in the tests tabulated below. In these tests the zirconium, in the form of commercial zirconium-silicon alloy, was added to the molten steel before casting, in the following manner:

The steels were melted in a basic lined electric steel-melting furnace, and when properly finished and ready for casting, zirconium-silicon was added to a portion of each steel in quantity corresponding to an addition of 0.20% Zr. To another ladle of the same steel, an identical quantity of silicon was added as ferrosilicon. The steels were then cast into ingots, forged, rolled and heat-treated simultaneously and in identical manner. All steels were tested in the air-cooled condition.

|                        | Heat 409 |         | Heat 411 |         | Heat 412 |         |
|------------------------|----------|---------|----------|---------|----------|---------|
|                        | No Zr    | With Zr | No Zr    | With Zr | No Zr    | With Zr |
| Carbon.....            | 0.52%    | 1.15%   | 0.29%    | 1.22%   | 0.24%    | 1.61%   |
| Manganese.....         |          |         |          |         |          |         |
| Yield point.....       | 68,700   | 61,600  | 57,800   | 62,200  | 48,800   | 46,200  |
| Tensile strength.....  | 118,500  | 113,600 | 92,300   | 90,000  | 95,400   | 92,600  |
| Elongation.....        | 18.5     | 20.5    | 27.0     | 28.2    | 24.0     | 25.7    |
| Reduction in area..... | 53.0     | 58.1    | 63.8     | 68.2    | 56.4     | 58.6    |
| Izod number.....       | 15.0     | 27.1    | 43.4     | 78.0    | 33.0     | 55.8    |
| Merit index.....       | 34.9     | 43.1    | 38.2     | 52.5    | 39.7     | 42.9    |

In connection with the foregoing table it may be explained that the Merit index is an arbitrary value which has been used by metallurgists in an attempt to grade steels, and is calculated from the data obtained in the so-called static tensile test. Naturally the significance of this index must be considered with respect to some particular application of the steel.

It will be noted that the shock resistance in the zirconium treated steels, as measured by the Izod test, has in these particular cases been increased by some 70 or 80% of its value in the untreated steels; and I have found a similar increase of at least 20%, and usually upward of 50%, for the entire range of compositions contemplated by this invention. It will also be noted that this increase in shock value has been secured without sacrifice of other valuable properties. Particularly in the higher carbon ranges, for example above

0.35%, or in steels of relatively lower ductility, the zirconium treatment brings about a pronounced improvement in ductility.

While the amounts of zirconium necessary to produce these effects are small, and although the manner in which zirconium acts has not as yet been certainly determined, it is regarded as preferable, if not essential, that the quantity of zirconium used should be sufficient so that a determinable amount exists in the finished steel. This was the case with each of the specific steels of which the properties are listed above.

My investigations indicate that the principal application of the invention will be to steels containing not more than about 0.7% carbon. It also appears that when the manganese content is toward the upper limit given, viz, at about 2.0%, the maximum carbon content referred to herein should not be incorporated. The best results have been obtained with steels wherein the sum of the carbon and manganese does not exceed 2.5%.

Steels having the chemical composition described herein acquire on air-cooling only a moderate degree of hardness and strength. Thus, in the specific examples tabulated, the tensile strength of the air-cooled steel does not exceed 125,000 pounds per square inch. The beneficial effect of zirconium on the ductility of steel is already known in connection with carbon and alloy steels heat-treated to impart to them a high degree of hardness and strength, but the prior art indicates that when the same steels are heat-treated to im-

part lower strength and hardness, as by quenching followed by drawing at 450° C. or higher, a content of zirconium does not increase the Izod number. In Patent No. 1,546,881 I have shown the effect of zirconium in raising the impact number of high phosphorus steels in the annealed condition. So far as I am aware the present invention constitutes the first case where a zirconium content has been shown to increase materially the Izod number of a steel having a normal phosphorus content and a tensile strength less than 125,000 pounds per square inch.

I claim:

1. The herein-described steel containing manganese substantially 1% to 2%; carbon below 1%; a substantial quantity of zirconium; and the hardness and strength characteristic of such a composition in the air-cooled condition.
2. The herein-described steel containing manganese substantially 1% to 2%; carbon below 1%; a substantial quantity of zirconium; a phosphorus content not above normal; and a tensile strength less than 125,000 pounds per square inch.
3. The herein-described steel containing manganese substantially 1% to 2%; carbon 0.35 to 0.70%; zirconium 0.15 to 0.50%; a phosphorus content not above normal; and a tensile strength less than 125,000 pounds per square inch.

In testimony whereof, I affix my signature.  
FREDERICK M. BECKET.